

# UNITED STATES PATENT OFFICE.

FREDERICK ROSE, OTTO MARCUS, AND ALBERT KLEMZ, OF PORTLAND, OREGON; SAID KLEMZ ASSIGNOR TO PAUL HAUCKE.

## KINDLING-BLOCK.

1,129,813.

Specification of Letters Patent. Patented Feb. 23, 1915.

No Drawing.

Application filed February 16, 1914. Serial No. 819,001.

To all whom it may concern:

Be it known that we, FREDERICK Rose, OTTO MARCUS, and ALBERT KLEMZ, citizens of the United States, residing at Portland, 5 in the county of Multnomah and State of Oregon, have invented certain new and useful Improvements in Kindling-Blocks, of which the following is a specification.

Our invention pertains to kindling blocks, 10 and has for its object to provide an article which may be readily ignited by the application of a lighted taper or the like and which possesses a fuel content in amount and character that will burn with a strong 15 blaze long enough to ignite ordinary fuel, without the use of specially prepared kindling.

It is further the object to provide such an article which is compact and reduced to the 20 smallest volume obtainable, and of a form and size convenient for use.

It is further an object to employ material 25 which ordinarily constitutes waste and to convert it into commercial article of universal use.

These objects are accomplished by use of the materials and in the manner hereinafter described.

In carrying out our invention we employ 30 wood which has been reduced to small particles, and prefer to use coarse shavings, such as may be obtained in shops or factories. These, which usually constitute waste, are sufficiently reduced to permit 35 their ready incorporation with the other materials to be employed; and they at the same time possess a value in fuel content which renders them particularly well adapted for the purpose.

In preparing the material, the moisture is 40 first driven from the wood in the form of shavings, by any usual drying operation, and seven parts of turpentine to 30 parts of shavings are then mixed with them, so that 45 every particle is covered by the turpentine. The shavings will then be allowed to stand long enough for the turpentine to penetrate into the wood and thus keep the wood in this inflammable substance. This will require 50 about eight hours, after which they will be

ready for the further steps in their preparation. Rosin in the proportion of 61 parts to 30 parts of the shavings will be heated until it is reduced to a thin liquid state, when two parts of sulfur will be added to it and 55 thoroughly mingled therewith. This liquid will be poured over the shavings prepared as above described, and mixed by grinding, or otherwise, until the ingredients are evenly distributed, and until the entire content has 60 reached the form of a plastic mass. This having been accomplished the material will be placed into molds of a form and size for convenient use, where it will be subjected to a high degree of pressure to shape it into 65 permanent blocks. Each of these blocks is designed to constitute sufficient kindling for any ordinary fuel, and it will produce an intense blaze for several minutes.

Blocks prepared in the manner above described, can be produced at an expense not greatly in excess of that of ordinary kindling, and it is always ready for use, without the need of the labor and disorder which 70 always attend the preparation of such kindling. The use of these blocks, moreover, is attended with perfect safety, and it will 75 thus be possible to dispense with the use of explosives for such purpose.

Having described our invention, what we 80 claim is—

1. An article of manufacture comprising a kindling block made of wood reduced to small parts steeped in turpentine and mixed with liquid rosin and sulfur in substantially 85 the proportions specified and pressed into blocks, substantially as described.

2. An article of manufacture comprising a combination of wood shavings, seven parts of turpentine, sixty-one parts of liquid rosin 90 and two parts of sulfur in block form.

In testimony whereof, we affix our signatures in the presence of two witnesses.

FREDERICK ROSE.  
OTTO MARCUS.  
ALBERT KLEMZ.

Witnesses:

E. EARL FEIKE,  
H. A. ARMSTRONG.

Copies of this patent may be obtained for five cents each, by addressing the "Commissioner of Patents, Washington, D. C."